



US006338762B1

(12) **United States Patent**  
Sato et al.

(10) **Patent No.:** US 6,338,762 B1  
(45) **Date of Patent:** Jan. 15, 2002

(54) **STAINLESS STEEL FOR USE IN ENGINE GASKETS AND A METHOD FOR MANUFACTURING THEREOF**

5,118,576 A 6/1992 Imae et al.  
5,624,504 A 4/1997 Miyakusu et al.

(75) Inventors: **Naoto Sato**, Funabashi; **Kazuhiko Adachi**, Jyoetsu; **Kenichi Goshokubo**, Niigata; **Takashi Katsurai**, Tochigi; **Shigeki Muroga**, Utsunomiya, all of (JP)

(73) Assignee: **Sumitomo Metal Industries, Ltd.**, Tokyo (JP)

(\*) Notice: Subject to any disclaimer, the term of this patent is extended or adjusted under 35 U.S.C. 154(b) by 0 days.

(21) Appl. No.: **09/564,649**

(22) Filed: **May 3, 2000**

**Related U.S. Application Data**

(63) Continuation of application No. PCT/JP99/04774, filed on Sep. 3, 1999.

(30) **Foreign Application Priority Data**

Sep. 4, 1998 (JP) ..... 10-251302  
(51) **Int. Cl.<sup>7</sup>** ..... **C21D 8/00**; C21D 9/00; C22C 38/40  
(52) **U.S. Cl.** ..... **148/325**; 148/327; 148/605; 148/610; 148/611; 148/651  
(58) **Field of Search** ..... 148/505, 610, 148/651, 611, 654, 325, 327

(56) **References Cited**

**U.S. PATENT DOCUMENTS**

4,564,566 A 1/1986 Jerlich et al.

**FOREIGN PATENT DOCUMENTS**

|    |               |         |
|----|---------------|---------|
| EP | 0273278       | 7/1988  |
| JP | 55-110758     | 8/1980  |
| JP | 63-162818 A * | 7/1988  |
| JP | 4-210453      | 7/1992  |
| JP | 4-214841      | 8/1992  |
| JP | 5-117813      | 5/1993  |
| JP | 5-279802      | 10/1993 |
| JP | 7-003406      | 1/1995  |
| JP | 7-278758      | 10/1995 |
| JP | 9-143633      | 6/1997  |

\* cited by examiner

*Primary Examiner*—Deborah Yee

(74) *Attorney, Agent, or Firm*—Burns, Doane, Swecker & Mathis, LLP

(57) **ABSTRACT**

An austenitic stainless steel for use in engine gaskets having a high fatigue strength and resistance to settlement and method of manufacture thereof. The austenitic stainless steel is prepared by cold rolling at least 40%, annealing at a temperature of 700° C. to 900° C. followed by temper rolling with a reduction of at least 40%. The metal structure obtained by annealing is a recovered unrecrystallized structure or a mixed structure of a recovered unrecrystallized structure and a recrystallized structure. The austenitic stainless steel includes at most 0.03% C, at most 1.0% Si, at most 2.0% Mn, 16.0% to 18.0% Cr, 6.0% to 8.0% Ni and up to 0.20% N.

**15 Claims, 1 Drawing Sheet**





*Fig. 1*



*Fig. 2*

## STAINLESS STEEL FOR USE IN ENGINE GASKETS AND A METHOD FOR MANUFACTURING THEREOF

This application claims priority under 35 U.S.C §§119 and/or 365 to Japanese patent application No. 251302 filed on Sep. 4, 1998; the entire content of which is hereby incorporated by reference.

This Application is a Continuation Application in the U.S.A. of PCT/JP99/04744, filed Sep. 3, 1999 in Japan.

### TECHNICAL FIELD

This invention relates to a stainless steel for use in engine gaskets and to a method for its manufacture, and particularly to a stainless steel for manufacturing an engine gasket which has excellent fatigue strength and excellent ability to maintain the shape of a bead portion when a stress load is applied for a long period and to a method for its manufacture.

The present invention also relates to a gasket which is obtained in that manner.

### TECHNICAL BACKGROUND

In the past, asbestos and the like have been used as gasket materials for use in apparatuses which increase in temperature, such as engines for use in automobiles or in boats. Recently, in response to increases in engine performance and moves to regulate the use of asbestos by laws, gaskets made of metal, i.e., metal gaskets, have come to be used.

Metal gaskets for use in engines must have various properties necessary for maintaining airtightness of joining surfaces. For example, metal gaskets used in the engines of automobiles, motorcycles, etc. must have properties enabling them to withstand the characteristic varying stresses of engines which are repeatedly applied in an atmosphere of combustion gas.

From the standpoint of sealing materials having similar uses, metal packings are increasingly used in place of O-rings wrapped in asbestos in response to moves to restrict the use of asbestos by laws as described above. In this case, a strip-shaped metal coil is wrapped into the shape of a cylinder, and it is formed into a donut-shaped O-ring to obtain a metal packing.

In the past, SUS301 (AISI301) type steel, which is a work hardened metastable austenite stainless steel which is given a high strength by simply performing cold working, was used as a raw material for these metal gaskets, metal packings, and the like.

For metal gaskets, a sheet having a thickness on the order of 0.1–0.4 millimeters is used as a raw material. In the case of a gasket for use in an engine head, for example, a bead is formed in the periphery of the combustion chamber and in the periphery of water supply holes and oil supply holes, and gas, water, and oil are sealed by the high pressure which is generated when clamping down of the bead is performed. For metal packings, a strip-shaped coil is wrapped into the shape of a cylinder, it is formed into the shape of a donut to form an O-ring, and it is used to maintain the airtightness of a joining surface.

Below, in this specification, such metal gaskets and metal packings will be generically referred to for convenience as “gaskets” or “engine gaskets”, and stainless steels used therein will be referred to as “stainless steels for engine gaskets”.

Even in the past, there were disclosures concerning gasket materials for use in engines in, for example, Japanese

Published Unexamined Patent Application No. HEI 4-214841, Japanese Published Unexamined Patent Application No. HEI 5-279802, and Japanese Published Unexamined Patent Application No. HEI 5-117813.

The stainless steels for engine gaskets disclosed in these official publications are all ones which are imparted with prescribed properties of fine, uniform recrystallized grains having an average grain diameter of at most 10 micrometers by performing finishing intermediate rolling at a reduction ratio of at least 50% followed by low temperature, short duration finish annealing.

### DISCLOSURE OF THE INVENTION

Namely, this existing technology relates to methods of manufacturing a stainless steel having excellent formability and fatigue properties characterized by using an austenitic stainless steel having components corresponding to SUS301, and by grain refining thereof by causing recrystallization by carrying out annealing at as low a temperature as possible.

However, at present, the properties of engines are continuously improving, and simultaneous with the trend towards higher engine output, the level of properties required of gasket materials has been increasing. However, there are various problems such as that it is difficult to obtain a material which has a fatigue strength which can adequately withstand this trend towards high engine output, that the final product has an inadequate hardness when a low carbon content is used, and that the shape maintaining ability of the portion which is subjected to working to form a bead when stress is applied for long periods (referred to below as resistance to settlement) is inadequate.

An object of this invention is to provide a stainless steel which is suitable for gaskets used in today's increasingly high performance engines and to a method for its manufacture.

Another object of this invention is to provide an engine gasket which can exhibit that type of excellent performance.

A more specific object of the present invention is to provide a stainless steel for engine gaskets which does not use materials requiring special components but which uses SUS301L stainless steel (roughly corresponding to low carbon AISI301) made of ordinary components and which has properties superior to those of existing materials, i.e., a high fatigue strength and excellent resistance to settlement, and to a method for its manufacture.

For example, a metal gasket used in an automotive engine or the like is subjected to working to form a bead. It is then mounted on an engine block, and it is repeatedly subjected to stress accompanying engine operation (explosions within the cylinders). Therefore, it is required to have adequate fatigue strength to resist this, and it is required to maintain the shape of the bead under such varying stress and to maintain a gas seal, i.e., it is required to have resistance to settlement.

An example of a steel which can cope with such conditions is a stainless steel corresponding to SUS301. As described above, such steels are generally used at present. Among the problems that were seen with such existing technology are the following:

1. In the case of a high carbon steel such as SUS301 (C: at most 0.15%), it is relatively easy to obtain a high hardness and to improve resistance to settlement. However, the more the hardness is increased, the more the fatigue strength ends up decreasing when working to obtain a bead is performed

in order to prepare an engine gasket, so it is difficult to obtain both fatigue strength and resistance to settlement. In addition, as a problem during the manufacturing stage, there is the possibility of carbides precipitating due to annealing, and there is a fear of a deterioration of corrosion resistance.

2. In the case of a low C content such as C: at most 0.03%, the corrosion resistance is excellent, and it is possible to increase the fatigue strength to a certain extent, but it is difficult to obtain an adequate hardness. For this reason, it is difficult to obtain an adequate resistance to settlement, and there is fear of a decrease in gas sealing properties.

3. Even higher fatigue strength and resistance to settlement are demanded due to increases in engine power, but with the existing technology using SUS301 type steel, it is difficult to achieve both at the same time, and at present, an increase in performance above existing levels is difficult.

The present inventors found that a sufficient level of hardness can be achieved even for a low carbon steel when temper rolling is carried out on a steel having a mixed structure of a recrystallized structure and a recovered, unrecrystallized structure, or a recovered, unrecrystallized structure corresponding to the structure before recrystallization occurs, which structure is prepared by finish annealing prior to temper rolling in order to reduce the influence of prior working. They also found that due to the remaining effects of previous working, if the strain due to working which is applied to the material after temper rolling has the same working rate as in an existing method, the deformation applied to crystal grains can be made large, and the effect of crystal grain boundaries in the structure on fatigue strength can be decreased. They additionally found that due to these synergistic effects, the fatigue strength can be markedly increased compared to that of existing materials.

The present invention is a stainless steel for engine gaskets characterized by comprising a temper rolled metal structure in the form of a recovered unrecrystallized structure or a mixed structure of a recovered unrecrystallized structure and a recrystallized structure. Namely, a stainless steel for engine gaskets according to the present invention comprises a martensite-containing structure obtained by temper rolling of a recovered unrecrystallized structure, or of a mixed structure of a recovered unrecrystallized structure and a recrystallized structure, both being obtained by annealing.

In this manner, a stainless steel for engine gaskets according to the present invention is one derived from a recovered unrecrystallized structure or a mixed structure of a recovered unrecrystallized structure and a recrystallized structure, both of which are obtained by finish annealing. The crystal structure of the metal structure at this time has a half-value width for the X-ray diffraction measured using CuK  $\alpha$  radiations for (220), (311) planes on austenite matrix of at least 0.15° and at most 0.35°.

From another standpoint, the present invention is a method of manufacturing a stainless steel plate for engine gaskets, in which cold rolling and annealing are repeatedly performed after hot rolling, and then temper rolling is performed, characterized in that the reduction during cold rolling carried out before finish annealing is at least 40%, the subsequently performed finish annealing is carried out in a temperature range of at least 700° C. and at most 800° C., and the metal structure is made a recovered unrecrystallized structure.

At this time, by carrying out finish annealing in a temperature range of at least 700° C. and at most 900° C., the metal structure can be made a recovered unrecrystallized

structure or a mixed structure of a recovered unrecrystallized structure and a recrystallized structure.

By making the reduction in the temper rolling after finish annealing at least 40%, the formation of martensite can be promoted.

Steels which are the object of the present invention are austenitic stainless steels, and particularly steels corresponding to SUS301(AISI301), and preferably, they are steels containing, by weight percent,

10 C: at most 0.03%, Si: at most 1.0%, Mn: at most 2.0%, Cr: at least 16.0% and at most 18.0%, Ni: at least 6.0% and at most 8.0%, and N: at most 0.20%.

From yet another standpoint, the present invention is an engine gasket made from a stainless steel having a temper rolled metal structure in which the metal structure is a recovered unrecrystallized structure or a mixed structure of a recovered unrecrystallized structure and a recrystallized structure.

20 In this manner, according to the present invention, a high hardness with a low C material which could not be obtained with existing technology is made possible, and an improvement in resistance to settlement can be obtained.

25 In addition, according to the present invention, using a stainless steel having components corresponding to generally known SUS301L, a stainless steel for engine gaskets having high fatigue strength and excellent resistance to settlement and a method for its manufacture are provided.

#### BRIEF EXPLANATION OF THE DRAWINGS

30 FIG. 1 is an explanatory view of the shape of a bead of a sample subjected to a fatigue test and a resistance to settlement test.

35 FIG. 2 is a view explaining the essentials of the fatigue test and the resistance to settlement test.

#### BEST MODE FOR CARRYING OUT THE INVENTION

An outline of the reasons for the limitations of an example of a suitable composition of a stainless steel used in the 40 present invention will be described below.

In general, a stainless steel used in the present invention can be SUS301L prescribed by JIS G 4305. Similar regulations are prescribed in U.S. Standards, or European Standards EN10088-1.

45 In a suitable mode of the present invention, the composition of such a stainless steel is prescribed as follows.

C is an austenite-forming element, it restricts delta-ferrite which is formed at high temperatures, and it is extremely effective for strengthening a martensite phase which is induced by cold working. However, if the C content is too high, work hardening becomes extreme, and during cold rolling it becomes difficult to regulate so as to achieve a target plate thickness, and manufacturability is worsened. In addition, there is a fear of deterioration in corrosion resistance accompanying precipitation of carbides due to annealing performed prior to temper rolling. Therefore, the range of C is preferably at most 0.03%. There is no particular lower limit, but in order to guarantee a prescribed strength, it is preferably at least 0.01%.

50 Si is added as a deoxidizing agent. In austenitic stainless steel, it is normally contained in an amount of about at most 1.0%. Therefore, in the present invention as well, Si is at most 1.0%.

Mn is an austenite-forming element. It is normally contained in an amount of about 2.0%, so in the present invention as well, Mn is at most 2.0%.

Cr is an indispensable component for guaranteeing a prescribed corrosion resistance. In order to impart a desired corrosion resistance and heat resistance, the amount is at least 13%. However, Cr is a ferrite-forming element, so if the amount is made too high, a large amount of delta-ferrite ends up being formed at high temperatures. On the other hand, if a large amount of an austenite-forming element is added to suppress a delta-ferrite phase, the austenite phase is stabilized at room temperature, and a high strength can not be obtained after cold working. From these standpoints, the range of Cr is preferably at least 16.0% and at most 18.0%.

Ni is an indispensable component for obtaining an austenite phase at high temperatures and at room temperature, but in the case of the present invention, it is added so as to obtain metastable austenite at room temperature, and so as to obtain an increase in strength due to work hardening accompanying the martensite transformation occurring during temper rolling.

If the amount of Ni is less than 6.0%, a large amount of delta-ferrite is formed at high temperatures, and it becomes easy for an excessive amount of work-induced martensite phase to be formed, hardening progresses, and elongation decreases. On the other hand, if the amount of Ni exceeds 8.0%, the austenite phase becomes stable, and it becomes difficult for a work induced martensite phase to form, so it is difficult to obtain sufficient hardness.

For this reason, the amount of Ni is at least 6.0% and at most 8.0%. From the standpoint of durability and heat resistance, it is also advantageous for the amount of Ni which is added to be at least 6.0%. However, if the added amount exceeds 8%, costs increase and the effect thereof saturates. From this standpoint as well, the amount of Ni is at least 6.0% and at most 8.0%.

Like C, N is an austenite-forming element, and it is an element which is effective for hardening a martensite phase and an austenite phase. In addition, compared to C, it does not readily form precipitates, so the addition of N is also effective from the standpoints of formability and fatigue strength. Also, it acts as a nucleus for recrystallization during annealing, and it is effective for refining the structure. However, if it is added in a large amount, it becomes a cause of blowholes, and during heat treatment, edge cracks are easily induced. Accordingly, in the present invention, it is preferably added in an amount of at most 0.20%. There is no particular lower limit thereon, but in order to obtain a desired effect, it is preferably at least 0.10%.

In a method of manufacturing a stainless steel according to the present invention, as a steel which meets these conditions, a stainless steel which corresponds to SUS301L set forth in generally known JIS G 4305 is applicable, but in this case, it is also possible for it to contain a certain amount of added elements, such as Mo, Cu, Nb, and the like other than those prescribed by JIS G 4305 with respect to SUS301L.

In the present invention, in the annealing which is carried out prior to temper rolling, the metal structure is made a recovered unrecrystallized crystal structure which occurs prior to recrystallization or a mixed structure of recrystallized grains and recovered unrecrystallized grains, and the amount of deformation of grains in the subsequent temper rolling is increased, and the effect of crystal grain boundaries on fatigue strength is made extremely small, as a result of which the fatigue strength is of course increased, and the ability to maintain shape (resistance to settlement) after working due to a high hardness being attained is enormously improved.

In the case of the present invention, it is not particularly necessary to perform aging such as is generally carried out, but if aging is additionally performed, a material of even higher strength is of course obtained.

In this manner, according to the present invention, it is possible to manufacture a gasket material having a higher fatigue strength and superior resistance to settlement compared to existing materials.

Here, the reasons for the limitations on a manufacturing method according to this invention will be described in more detail.

The structural state of a stainless steel used in this invention is essentially an austenite structure at the time of solution treatment. In the rolling performed prior to finish annealing prior to temper rolling of this steel, namely during finishing intermediate rolling, cold rolling with a reduction of at least 40% and preferably from 40 to 70% is carried out. As a result, in finish annealing prior to temper rolling, by performing finish annealing at a relatively low annealing temperature, i.e., in a temperature range of at least 700°C. and at most 800°C. or at least 700°C. and at most 900°C., a recovered unrecrystallized structure or a mixed structure of recrystallized grains and a recovered unrecrystallized structure is obtained, and then by carrying out cold working of at least 40% in the subsequently performed temper rolling, a metal gasket material having sufficient properties can be obtained.

The soaking time during finish annealing at this time is preferably from 0 to 60 seconds. If it exceeds 60 seconds, there is the possibility of an entirely recrystallized structure.

Here, the finish annealing prior to temper rolling is particularly restricted to at least 700°C. and at most 800°C. or at least 700°C. and at most 900°C. This is because if the temperature is less than 700°C., a long time is required for recovery in order to decrease the effects of previous working, which is not industrially practical. If the temperature exceeds 800°C., a recrystallized structure begins to form. In addition, if the temperature exceeds 900°C., the structure ends up being almost entirely a recrystallized structure.

There is no particular limit on the percentage of recovered unrecrystallized grains, but in order to obtain necessary properties, it is desirable that it be at least 50%.

In this manner, according to the present invention, due to finish annealing carried out prior to temper rolling, the metal structure is made a recovered unrecrystallized structure or a mixed structure of recrystallized grains and a recovered unrecrystallized structure. The reason for this is to increase the work induced strain applied to the material after temper rolling which is subsequently performed because of the remaining effects of previous working, to increase the deformation which is thereby applied to grains, to make the effect on crystal grain boundaries as small as possible, and to improve the fatigue strength after bead formation. In addition, this is in order to obtain a material of higher hardness, and to improve the resistance to settlement of the bead portion.

The finish annealing can be carried out on an industrial scale using a continuous annealing equipment.

The above-described recovered unrecrystallized structure or the mixed structure of recrystallized grains and a recovered unrecrystallized structure is one having a crystal structure in which each half-value width of (220), (311) on austenite matrix is at least 0.15° and at most 0.35° by X-ray diffraction measured using CuK $\alpha$  radiation.

The metal structure which is obtained at this time can be made entirely into a recovered unrecrystallized structure by

making the annealing temperature during finish annealing 700 to 800° C.

After finish annealing, temper rolling is carried out. Due to the remaining effects of prior working, a rolling reduction of at least 40% is sufficient, and a large increase in fatigue strength and a high strength can be obtained. In the present invention, the rolling reduction of this temper rolling can be set to various values within the range of at least 40%, but even with the same rolling reduction as used with existing steels, a material of higher fatigue strength and superior resistance to settlement can be obtained.

In this manner, according to the present invention, it is possible to provide the properties necessary for an engine gasket material, so aging which is generally carried out to obtain an increase in strength is not necessary, but if aging is performed, a material of even higher performance can of course be obtained.

The metastable austenite stainless steel which is the object of the present invention exhibits an austenite phase in solid solution, so the manufacturing steps prior to finishing intermediate rolling performed prior to finish annealing can be the same as for existing materials.

Next, the effects of the present invention will be shown in greater detail by an example.

#### EXAMPLE

Table 1 shows the components of a stainless steel used in this example.

Table 2 shows the mechanical properties, the half-value width of X-ray diffraction, the fatigue strength, and the resistance to settlement when the rolling reduction in cold rolling performed prior to finish annealing preceding temper rolling, the annealing conditions, and the temper rolling reduction were varied.

Each of the steels shown in FIG. 1, i.e., the steels of the present invention (1-3), and the comparative steels (4-6) were melted in an ordinary atmospheric melting furnace, were subjected to hot rolling followed by cold rolling and annealing, and then were formed by temper rolling to a thickness of 0.20 millimeters. Samples were then collected from the steels. In each case, finish annealing was carried out by maintaining the steels for 10 seconds (soaking time) after

a set temperature was reached. The details of the rolling reduction in finishing intermediate rolling prior to finish annealing, the annealing conditions, and the temper rolling reduction for each steel are shown in Table 2.

The collected samples were subjected to a tensile test and a hardness test to measure their mechanical properties, and they were subjected to a fatigue test and a settlement test to evaluate their fatigue strength and their resistance to settlement.

FIG. 1 is a schematic perspective view showing a test piece for the fatigue test and the resistance to settlement test and particularly the shape of the bead.

FIG. 2 is a view for explaining the essentials of the repeated compression and load release carried out in the fatigue test and the resistance to settlement test.

In this example, the bead had a width of 2.5 millimeters and a height of 0.25 millimeters. In the fatigue test, a test piece on which this bead portion was formed was repeatedly loaded from above and below as shown in FIG. 2, and after compression and release of a load were repeated  $10^6$  times, the fatigue strength was evaluated based on whether cracks were formed in the test piece. Those with no change are shown by a circle, and those which suffered cracking or fracture are indicated by an X.

Similarly, in the resistance to settlement test, compression and release of load were repeated  $10^5$  times, after which those having a ratio  $(h/h_0)$  of the remaining bead height  $h$  to the initial bead height  $h_0$  of at least 0.5 were evaluated as good and those of less than 0.5 were evaluated as bad, and are respectively shown by a circle and by an X.

Those having good formability when the formation of a bead shown in FIG. 1 was carried out are indicated by a circle, and those in which cracking or fracture took place are indicated by an X.

In order to determine the state of the metal structure of the material obtained after finish annealing, measurement of the half-value width by X-ray diffraction using CuK  $\alpha$  radiation was carried out on the materials after finish annealing.

The results are collectively shown in Table 2.

TABLE 1

| Steel<br>Number | C | Si     | Mn   | S    | Ni    | Cr    | N      | Nb     | Mo    | Cu   | Remainder: Fe (weight %) |                        |
|-----------------|---|--------|------|------|-------|-------|--------|--------|-------|------|--------------------------|------------------------|
|                 |   |        |      |      |       |       |        |        |       |      | Remarks                  |                        |
| Present         | 1 | 0.023  | 0.59 | 1.61 | 0.002 | 6.70  | 17.22  | 0.115  | 0.068 | 0.28 | 0.31                     | Corresponds to SUS301L |
| Invention       | 2 | 0.011  | 0.52 | 1.43 | 0.001 | 6.65  | 17.89  | 0.124  | 0.071 | 0.20 | 0.18                     |                        |
|                 | 3 | 0.013  | 0.48 | 1.35 | 0.003 | 7.08  | 16.28  | 0.159  | 0.065 | 0.19 | 0.20                     |                        |
| Comparative     | 4 | 0.099* | 0.57 | 0.81 | 0.003 | 6.74  | 17.01  | 0.061* | 0.007 | 0.26 | 0.27                     | Corresponds to SUS301  |
|                 | 5 | 0.053* | 0.37 | 0.92 | 0.002 | 8.02* | 18.19* | 0.034* | 0.009 | 0.21 | 0.19                     | Corresponds to SUS304  |
|                 | 6 | 0.017  | 0.33 | 0.98 | 0.002 | 9.01* | 18.16* | 0.031* | 0.008 | 0.18 | 0.18                     | Corresponds to SUS304L |

(Note)

\*: Indicates outside the range prescribed by the present invention.

TABLE 2

| Example Number    | Steel Number | Manufacturing Conditions |                         |                    |                             | Results                  |                |                      |                  |               |                          |             |
|-------------------|--------------|--------------------------|-------------------------|--------------------|-----------------------------|--------------------------|----------------|----------------------|------------------|---------------|--------------------------|-------------|
|                   |              | Finish Rolling (%)       | Finish Annealing (° C.) | Temper Rolling (%) | 0.2% Yield Strength (N/mm²) | Tensile Strength (N/mm²) | Elongation (%) | Half-Value Width (°) | Fatigue Strength | Hardness (Hv) | Resistance to Settlement | Formability |
| Present Invention | 1            | 1                        | 50                      | 800                | 50                          | 1290                     | 1424           | 8.0                  | 0.20             | ○             | 454                      | ○ ○         |
|                   | 2            | 2                        | 50                      | 800                | 50                          | 1285                     | 1422           | 8.3                  | 0.20             | ○             | 451                      | ○ ○         |
|                   | 3            | 3                        | 50                      | 800                | 50                          | 1284                     | 1420           | 8.3                  | 0.20             | ○             | 453                      | ○ ○         |
|                   | 4            | 1                        | 40                      | 800                | 50                          | 1289                     | 1427           | 8.0                  | 0.21             | ○             | 450                      | ○ ○         |
|                   | 5            | 1                        | 60                      | 800                | 50                          | 1302                     | 1441           | 7.4                  | 0.23             | ○             | 456                      | ○ ○         |
|                   | 6            | 1                        | 50                      | 700                | 50                          | 1390                     | 1504           | 4.6                  | 0.35             | ○             | 458                      | ○ ○         |
|                   | 7            | 1                        | 50                      | 900                | 50                          | 1285                     | 1410           | 9.8                  | 0.18             | ○             | 440                      | ○ ○         |
|                   | 8            | 1                        | 50                      | 800                | 40                          | 1274                     | 1408           | 9.2                  | 0.20             | ○             | 450                      | ○ ○         |
|                   | 9            | 1                        | 50                      | 800                | 60                          | 1301                     | 1431           | 7.7                  | 0.20             | ○             | 457                      | ○ ○         |
|                   | 10           | 4                        | 40                      | 800                | 40                          | 1431                     | 1675           | 1.9                  | 0.42*            | —             | 520                      | — X         |
| Comparative       | 11           | 5                        | 40                      | 800                | 40                          | 1390                     | 1514           | 1.8                  | 0.41*            | X             | 434                      | X ○         |
|                   | 12           | 6                        | 40                      | 800                | 40                          | 1262                     | 1389           | 4.4                  | 0.40*            | X             | 391                      | X ○         |
|                   | 13           | 1                        | 30*                     | 800                | 50                          | 1406                     | 1525           | 3.6                  | 0.38*            | —             | 460                      | — X         |
|                   | 14           | 1                        | 50                      | 675*               | 50                          | 1418                     | 1541           | 2.8                  | 0.39*            | —             | 462                      | — X         |
|                   | 15           | 1                        | 50                      | 925*               | 50                          | 1250                     | 1393           | 11.8                 | 0.14*            | X             | 429                      | X ○         |

(Note)

\*: Indicates outside the range prescribed by the present invention.

## Possibility of Industrial Use

According to the present invention, a stainless steel for use in engine gaskets having superior fatigue strength and resistance to settlement is obtained. A manufacturing method according to this invention reduces the effects of prior working on the metal structure after finish annealing performed prior to temper rolling, and by making a recovered unrecrystallized structure prior to the occurrence of recrystallization or a mixed structure of recrystallized grains and a recovered unrecrystallized structure, compared to other manufacturing methods using existing metal gasket materials in the form of SUS301-type steels, it is possible to manufacture a material having both a high fatigue strength and resistance to settlement. A manufacturing method for a stainless steel for engine gaskets of this type according to the present invention having such properties can be carried out using a stainless steel with generally well-known components using existing equipment, and finish annealing prior to temper rolling can be easily carried out on a continuous annealing line, so the manufacturing method provides excellent economy.

What is claimed is:

1. An austenitic stainless steel for use in engine gaskets characterized by having a structure in which the half-value width by X-ray diffraction measured using CuK  $\alpha$  radiation for (220), (311) planes on austenite matrix is at least 0.15° and at most 0.35°, and wherein the stainless steel contains, by weight percent, C: at most 0.03%, Si: at most 1.0%, Mn: at most 2.0%, Cr: at least 16.0% and at most 18.0%, Ni: at least 6.0% and at most 8.0% and N: at most 0.20%.
2. An austenitic stainless steel for use in engine gaskets characterized by having a temper rolled metal structure which is a recovered unrecrystallized structure or a mixed structure of a recovered unrecrystallized structure and a recrystallized structure, and wherein the stainless steel contains, by weight percent, C: at most 0.03%, Si: at most 1.0%, Mn: at most 2.0%, Cr: at least 16.0% and at most 18.0%, Ni: at least 6.0% and at most 8.0%, and N: at most 0.20%.
3. An austenitic stainless steel for use in engine gaskets characterized by having a martensite-containing metal structure obtained by performing a temper rolling after obtaining

25 by annealing a recovered unrecrystallized structure or a mixed structure of a recovered unrecrystallized structure and a recrystallized structure, and wherein the stainless steel contains, by weight percent,

C: at most 0.03%, Si: at most 1.0%, Mn: at most 2.0%, Cr: at least 16.0% and at most 18.0%, Ni: at least 6.0% and at most 8.0%, and N: at most 0.20%.

30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 82

**11**

8. A gasket made of an austenitic stainless steel as claimed in claim 1.
9. A gasket made of an austenitic stainless steel as claimed in claim 2.
10. A gasket made of an austenitic stainless steel as claimed in claim 3.
11. The austenitic stainless steel as claimed in claim 1, wherein N is 0.10 to 0.20%.
12. The austenitic stainless steel as claimed in claim 2, wherein N is 0.10 to 0.20%.
13. The austenitic stainless steel as claimed in claim 3, wherein N is 0.10 to 0.20%.

**12**

14. A method of manufacturing an austenitic stainless steel for use in engine gaskets as claimed in claim 4 wherein the stainless steel contains, by weight percent, C: at most 0.03%, Si: at most 1.0%, Mn: at most 2.0%, Cr: at least 16.0% and at most 18.0%, Ni: at least 6.0% and at most 8.0%, and N: at most 0.20%.
15. A method of manufacturing an austenitic stainless steel for use in engine gaskets as claimed in claim 4, wherein N is 0.10 to 0.20%.

\* \* \* \* \*

UNITED STATES PATENT AND TRADEMARK OFFICE  
**CERTIFICATE OF CORRECTION**

PATENT NO. : 6,338,762 B1  
DATED : January 15, 2002  
INVENTOR(S) : Naoto Sato et al.

Page 1 of 1

It is certified that error appears in the above-identified patent and that said Letters Patent is hereby corrected as shown below:

Title page.

Assignee information is corrected to read:

-- [73] Assignees: **Sumitomo Metal Industries, Ltd.,**  
Osaka (JP)

**Honda Giken Kogyo Kabushiki Kaisha**  
Tokyo (JP) --

Signed and Sealed this

Twenty-ninth Day of October, 2002

Attest:



Attesting Officer

JAMES E. ROGAN  
Director of the United States Patent and Trademark Office